

## UNITED STATES PATENT OFFICE

2,640,776

SENSITIZED PHOTOGRAPHIC EMULSION  
CONTAINING COLOR COUPLERSJohn Spence and Burt H. Carroll, Rochester,  
N. Y., assignors to Eastman Kodak Company,  
Rochester, N. Y., a corporation of New JerseyNo Drawing, Application August 29, 1947,  
Serial No. 771,380

11 Claims. (Cl. 95-7)

1

This invention relates to spectrally (optically) sensitized photographic silver halide emulsions containing color couplers.

In general, in subtractive color photography blue, green and red sensitive photographic silver halide emulsions are employed. The green and red sensitivities are obtained by the use of sensitizing dyes adsorbed to the silver halide grains. When couplers or dispersions of couplers are incorporated in the dye-sensitized emulsions, it is necessary that they do not alter the spectral (optical) sensitization produced by the dyes.

With the very great majority of sensitizing dyes, the molten sensitized silver halide emulsions in combination with the color couplers or dispersions of color couplers are not stable enough to permit the obtaining of uniform sensitivity throughout the period of coating; the emulsions losing the sensitivity conferred by the dye to a considerable degree during the coating operation.

We have now found that certain combinations of silver halide emulsions sensitizing dyes and color couplers are, in fact, stable and that the melted emulsions can be coated without appreciable loss in dye-sensitivity.

It is, accordingly, an object of our invention to provide stable combinations of silver halide emulsions sensitizing dyes and color couplers. A further object is to provide a process for preparing such combinations. Still other objects will become apparent hereinafter.

In accordance with our invention we prepare an emulsion for color photography comprising a red-sensitive silver halide emulsion containing a color-former (coupler) for the cyan image (i. e. a color-former capable of forming a quinoneimine dye with a phenylenediamine developer), said red-sensitive emulsion being sensitized with at least one sensitizing dye selected from the group consisting of those dyes represented by the following general formulas:



and R<sub>4</sub> each represents a member selected from the group consisting of a hydrogen atom and an alkyl group containing from 1 to 4 carbon atoms, e. g. methyl, ethyl, n-propyl, isobutyl and n-butyl,

5 Z and Z<sub>1</sub> each represents non-metallic atoms necessary to complete a heterocyclic nucleus selected from the group consisting of heterocyclic nuclei of the benzothiazole series, heterocyclic nuclei of the benzoselenazole series, heterocyclic nuclei of the naphthothiazole series and heterocyclic nuclei of the naphthoselenazole series, e. g. the benzothiazole nucleus, the 5-methylbenzothiazole nucleus, the 5-methoxybenzothiazole nucleus, the 5-ethylbenzothiazole nucleus, the 5-ethoxybenzothiazole nucleus, the 5-phenylbenzothiazole nucleus, the 5-chlorobenzothiazole nucleus, the 5-bromobenzothiazole nucleus, the benzoselenazole nucleus, the 5-chlorobenzoselenazole nucleus, the  $\alpha$ -naphthothiazole nucleus, the  $\beta$ -naphthothiazole nucleus, the  $\alpha$ -naphthoselenazole nucleus, the  $\beta$ -naphthoselenazole nucleus, etc., R<sub>1</sub> and R<sub>3</sub> each represents an alkyl group containing from 1 to 2 carbon atoms, i. e. methyl and ethyl, R<sub>2</sub> represents a monocyclic aryl group of the benzene series, e. g. phenyl, p-methoxyphenyl, m-tolyl, p-chlorophenyl, p-ethoxyphenyl, p-tolyl, p-bromophenyl, and X represents an anion, e. g. chloride, bromide, iodide, methylsulfate, ethylsulfate, p-toluenesulfonate, benzenesulfonate, acetate, propionate, thiocyanate, perchlorate, etc.

In accordance with our invention, we prepare a yellow-green sensitive silver halide emulsion containing a color-former (coupler) for the magenta image (i. e. a color-former capable of forming an azomethine dye with a phenylenediamine developer), said yellow-green sensitive silver halide emulsion being sensitized with at least one sensitizing dye selected from the group consisting of those dyes represented by the following general formulas:



wherein D and D<sub>1</sub> each represents a divalent aliphatic hydrocarbon radical containing from 1 to 4 carbon atoms, e. g. methylene, ethylene, ethylidene, trimethylene, tetramethylene, etc., R



wherein R<sub>4</sub> and R<sub>5</sub> each represents an alkyl group containing from 1 to 4 carbon atoms, e. g. methyl, ethyl, n-propyl, n-butyl, isobutyl, etc., X<sub>1</sub> represents an anion, e. g. benzenesulfonate, p-toluenesulfonate, chloride, bromide, iodide, perchlorate, methylsulfate, ethylsulfate, thiocyanate, acetate, propionate, etc., D<sub>2</sub> and D<sub>3</sub> each represents a divalent hydrocarbon radical containing from 1 to 4 carbon atoms, e. g. methylene, ethylene, ethylidene, trimethylene, tetramethylene, etc., and Z<sub>3</sub> represents the non-metallic atoms necessary to complete a heterocyclic nucleus of the quinoline series, e. g. the quinoline nucleus, the 6-methylquinoline nucleus, the 6-ethylquinoline nucleus, the 6-methoxyquinoline nucleus, the 6-ethoxyquinoline nucleus, the 6-chloroquinoline nucleus, etc.

In the preparation of photographic elements for color photography employing our new emulsions, any of the customary procedures can be used. Thus, the emulsions can be coated on a support as separate layers, e. g. a support (of cellulose acetate film, resin film, paper, etc.) can be coated with a layer of the red-sensitive emulsion containing a color former (as described above) and upon this, a layer of the yellow-green sensitive emulsion containing a color former (as described above) can be coated. Upon the yellow-green sensitive layer, a yellow filter layer can then be coated and upon the filter layer a layer of a blue sensitive emulsion containing a color-former which produces a yellow image or picture. Typical multi-emulsion photographic elements (involving color-formers in the emulsion) to which our invention is applicable are described in United States Patents 1,055,155, dated March 4, 1913; 2,304,940, dated December 15, 1942, and 2,322,027, dated June 15, 1943.

Our invention is also applicable to color photographic emulsion material wherein the emulsions are mixed instead of disposed in separate layers. Moreover, our invention is also applicable for producing single emulsions containing color-formers for making component color pictures. In addition to the sensitizing dyes and color-formers the emulsions employed in our invention can also contain the usual additions to emulsions, e. g. stabilizers, etc.

Our invention is especially useful where the emulsions contain, in addition to a color-former, a dispersing agent for the color-former, e. g. the water-insoluble but water-permeable materials set forth in U. S. Patents 2,304,940 and 2,322,027, such as water-insoluble but water-permeable cellulose esters, e. g. water-insoluble, but water-permeable cellulose acetate, cellulose acetate-phthalate, cellulose nitrate, etc., water-insoluble, but water-permeable cellulose ethers, water-in-

soluble but water-permeable natural and synthetic resins, high-boiling, substantially water-insoluble crystalloidal materials, such as N-n-amyolphthalimide, tetrahydrofurfuryl benzoate, triphenyl phosphate, n-butyl sulfone, ethyl-N,N-di-n-butylcarbamate, ethyl-N-phenylcarbamate, tetrahydrofurfuryl succinate, ethyl benzyl malonate, methyl phthalate, n-butyl phthalate, n-amyI phthalate,  $\beta$ -methoxyethyl phthalate,  $\beta$ -ethoxyethyl phthalate,  $\beta$ -butoxyethyl phthalate, butyl o-methoxybenzoate, n-hexyl benzoate, benzophenone, p - sec - amyIbenzophenone, tricresyl phosphate, diphenyl mono-p-tert. butyl phenyl phosphate, monophenyl di-o-chlorophenyl phosphate, tri-o-phenylphenyl phosphate, p-toluenesulfonyl methyl-o-toluidine, p-toluenesulfonyl dimethylamide, p,p'-di-n-amyIbenzenesulfonamide, p-toluenesulfonyl di-n-butyl amide, N,N'-diethyl-N,N'-diphenyl urea, N,N-di-n-butyl urea, etc.

Our invention is especially useful with emulsions in which the color-former is dispersed in one or more of the aforesaid substantially water-insoluble, high-boiling crystalloidal materials. These crystalloidal materials are organic and have boiling points above about 175° C. These crystalloidal materials have a high solvent action for the color-formers and for the dyes formed therefrom and are permeable to photographic processing solutions. These crystalloidal materials have been referred to as "oil formers" because they have the property of producing an oily or liquid solution when mixed with the coupler, even though the coupler is a solid. The crystalloidal materials are generally liquid at ordinary temperatures or low melting solids (below 100° C.). The most useful compounds contain one or more polar groups such as halogen, hydroxyl, carboxylic acid, amide, ketone, etc.

The following couplers are suitable for use in our invention. It is to be understood that this list is not exhaustive, but merely to typify compounds which may be used.

#### Couplers producing cyan images

- 45 5-(p-amylphenoxybenzenesulfonamino)-1-naphthol  
 5-(N - benzyl - N - naphthalenesulfonamino)-1-naphthol  
 50 5-(n-benzyl-N-n-valerylamino)-1-naphthol  
 5-caproylamino-1-naphthol  
 2-chloro-5-(N-n-valeryl - N - p- isopropylbenzylamino)-1-naphthol  
 55 2,4 - dichloro-5-(p-nitrobenzoyl- $\beta$ -o-hydroxyethylamino)-1-naphthol  
 2,4-dichloro-5-palmithylamino-1-naphthol  
 2,2'-dihydroxy-5,5'-dibromostilbene  
 5-diphenylethersulfonamido-1-naphthol  
 1-hydroxy-2-(N-isoamyl-N-phenyl)naphthamide  
 1-hydroxy-2-(N-p-sec. amyIphenyl)-naphthamide  
 60 8 - hydroxy-1- $\alpha$ -naphthoyl - 1,2,3,4 - tetrahydroquinoline  
 2-lauryl-4-chlorophenol  
 1-naphthol-2-carboxylic- $\alpha$ -naphthalide  
 1-naphthol-5-sulfo-cyclohexylamide  
 5-phenoxyacetamino-1-naphthol  
 5- $\beta$ -phenylpropionylamino-1-naphthol  
 Monochlor-5-(N- $\gamma$ -phenylpropyl-N-p-sec.-amyIbenzoylamino)-1-naphthol  
 2-acetylamin-5-methylphenol  
 2-benzoylamino-3,5-dimethylphenol  
 2- $\alpha$ (p - tert. amyIphenoxy) - n - butyrylamino-5-methylphenol

- 5  
 2-*a*(*p* - tert. amylphenoxy) - *n* - butyrylamino-4-chloro-5-methylphenol  
 2-(*p'* - tert. amylphenoxy - *p* - benzoyl)amino-4-chloro-5-methylphenol  
 2-(4'' - tert. amyl-3'-phenoxybenzoylamino) - 3,5-dimethyl-1-phenol  
 2-phenylacetylamino-4-chloro-5-methylphenol  
 2-benzoylamino-4-chloro-5-methylphenol  
 2-anilinoacetylamino-4-chloro-5-methylphenol  
 2-{4' - [*a*(4'' - tert. amylphenoxy) - *n* - butyryl-amino] - benzoylamino} - 4 - chloro-5-methylphenol  
 2-[4'-3''' - (4'' - tert. amylphenoxy) benzoylamino] benzoylamino-4-chloro-5-methylphenol  
 2-*p*-nitrobenzoylamino-4-chloro-5-methylphenol  
 2-*m*-aminobenzoyl-4-chloro-5-methylphenol  
 2-acetamino-4-chloro-5-methylphenol  
 2(4'-sec. amylbenzamino) - 4-chloro-5-methylphenol  
 2(4'-*n*-amyloxybenzamino) - 4-chloro-5-methylphenol  
 2-(4'-phenoxybenzoylamino) phenol  
 2-(4'' - tert. amyl-3'-phenoxybenzoylamino) phenol  
 2 - [*a* - (4' - tert. butylphenoxy) propionylamino] - phenol  
 2-[*a* - (4' - tert. amyl) phenoxypropionylamino] - phenol  
 2-[N-methyl-*N*-(4'' - tert. amyl-3'-phenoxybenzoylamino)]phenol  
 2-(4'' - tert. amyl-3'-phenoxybenzoylamino) - 3-methyl-1-phenol  
 2-(4'' - tert. amyl-3'-phenoxybenzoylamino) - 6-methyl-1-phenol  
 2-(4'' - tert. amyl-3'-phenoxybenzoylamino) - 3,6-dimethylphenol  
 2,6-di-(4'' - tert. amyl-3'-phenoxybenzoylamino) - 1-phenol  
 2 - *a* - (4' - tert. amylphenoxy) butyrylamino - 1-phenol  
 2-(4'' - tert. amyl-3'-phenoxybenzoylamino) - 3,5-dimethyl-1-phenol  
 2-[*a* - (4' - tert. amylphenoxy) - *n* - butyrylamino] - 5-methyl-1-phenol  
 2-(4'' - tert. amyl-3'-phenoxybenzoylamino) - 4-chloro-1-phenol  
 3 - [*a* - (4' - tert. amylphenoxy) *n* - butyrylamino] - 6-chlorophenol  
 3-(4'' - tert. amyl-3'-phenoxybenzoylamino) phenol  
 2-[*a* - (4' - tert. amylphenoxy) - *n* - butyrylamino] - 6-chlorophenol  
 3-[*a* - (4' - tert. amylphenoxy) - *n* - butyrylamino] - 4-chlorophenol  
 3-[*a* - (4' - tert. amylphenoxy) - *n* - butyrylamino] - 5-chlorophenol  
 3-[*a* - (4' - tert. amylphenoxy) - *n* - butyrylamino] - 2-chlorophenol  
 2-[*a* - (4' - tert. amylphenoxy) butyrylamino] - 5-chlorophenol  
 2-(4'' - tert. amyl-3'-phenoxybenzoylamino) - 3-chlorophenol  
 5-benzene sulfonamino-1-naphthol  
 2,4-dichloro-5-benzenesulfamino-1-naphthol  
 2,4-dichloro-5-(*p*-toluenesulfamino)-1-naphthol  
 5-(1,2,3,4-tetrahydronaphthalene-6-sulfamino) - 1-naphthol  
 2,4-dichloro-5-(4'-bromodiphenyl-4-sulfonamino)-1-naphthol  
 5-(quinoline-5-sulfamino)-1-naphthol

1947, can be used as couplers for the cyan image, e. g.



etc.

#### Couplers producing magenta images

- 30 1-p-sec. amylphenyl-3-*n*-amyl-5-pyrazolone  
 2-cyanoacetyl - 5 - (p-sec. amylbenzoylamino) - coumarone  
 2-cyanoacetylcoumarone - 5 - (*n*-*n*-amyl-p-sec. amylsulfanilide)  
 35 2-cyanoacetylcoumarone - 5 - (*N*-*n*-amyl-p-tert. amylsulfanilide)  
 2-cyanoacetylcoumarone - 5 - sulfon-*N*-*n*-butyl-anilide  
 2-cyanoacetyl-5-benzoylamino-coumarone  
 40 2-cyanoacetylcoumarone-5-sulfondimethylamide  
 2-cyanoacetylcoumarone-5-sulfon-*N*-methylanilide  
 2-cyanoacetylnaphthalene sulfon-*N*-methylanilide  
 45 2-cyanoacetylcoumarone-5-(*N*- $\gamma$ -phenylpropyl) - p-tert. amylsulfanilide  
 1-p-laurylphenyl-3-methyl-5-pyrazolone  
 1- $\beta$ -naphthyl-3-*n*-amyl-5-pyrazolone  
 1-p-nitrophenyl-3-*n*-amyl-5-pyrazolone  
 50 1-p-phenoxyphenyl-3-*n*-amyl-5-pyrazolone  
 1-phenyl-3-*n*-amyl-5-pyrazolone  
 1,4-phenylene bis-3-(1-phenyl-5-pyrazolone)  
 1-phenyl-3-acetylamino-5-pyrazolone  
 1-phenyl-3-propionylamino-5-pyrazolone  
 55 1-phenyl-3-*n*-valerylamino-5-pyrazolone  
 1-phenyl-3-chloroacetylamino-5-pyrazolone  
 1-phenyl-3-dichloroacetylamino-5-pyrazolone  
 1-phenyl-3-benzoylamino-5-pyrazolone  
 60 1-phenyl-3-(*n*-aminobenzoyl)amino-5-pyrazolone  
 1-phenyl-3-(p-sec. amylbenzoylamino)5-pyrazolone  
 1-phenyl-3-diethylbenzoylamino-5-pyrazolone  
 65 1-phenyl-3- $\beta$ -naphthoylamino-5-pyrazolone  
 1-phenyl-3-phenylcarbamylamino-5-pyrazolone  
 1-phenyl-3-palmitylamino-5-pyrazolone  
 1-phenyl-3-benzenesulfonylamino-5-pyrazolone  
 1-(*p*-phenoxyphenyl) - 3 - (p-tert. amyloxybenzoyl)amino-5-pyrazolone

Of course, for photographic elements involving a blue-sensitive, as well as a yellow-green sensitive, and a red-sensitive emulsion, color-formers which produce yellow images are employed and

any of the color-formers producing yellow images can be used, e. g.

*Couplers producing yellow images*

- N-amyl-p-benzoylacetaminobenzenesulfonate  
 N-(4-anisoylacetaminobenzenesulfonyl)-N-benzyl-m-toluidine  
 N-(4-benzoylacetaminobenzenesulfonyl)-N-benzyl-m-toluidine  
 N-(4-benzoylacetaminobenzenesulfonyl)-N-n-amyl-p-toluidine  
 N-(4-benzoylacetaminobenzenesulfonyl)-N-benzylaniline  
 $\omega$ -(p-Benzoylbenzoyl) acetanilide  
 $\omega$ -Benzoylacet-2,5-dichloroanilide  
 $\omega$ -Benzoyl-p-ace. amylacetanilide  
 N,N'-di( $\omega$ -benzoylacetyl)-p-phenylenediamine  
 N,N'-di-(acetoacetamino)-diphenyl  
 4,4'-di-(Acetoacetamino)-3,3'-dimethyldiphenyl  
 p,p'-di-(Acetoacetamino)-diphenylmethane  
 Ethyl-p-benzoylacetaminobenzenesulfonate  
 Nonyl-p-benzoylacetaminobenzenesulfonate  
 N-phenyl-N'-(p-acetoxycetaminophenyl)-urea  
 n-Propyl-p-benzoylacetaminobenzenesulfonate  
 acetoacetpiperide  
 $\omega$ -Benzoylacetpiperide  
 N( $\omega$ -benzoylacetyl)-1,2,3,4-tetrahydroquinoline  
 N-( $\omega$ -benzoylacetyl)morpholine

The aforesaid couplers give color development with color developers, such as N,N-dimethyl-p-phenylenediamine, N,N-diethyl-p-phenylenediamine, N-carbamidomethyl-N-methyl-p-phenylenediamine, N<sup>4</sup>-carbamidomethyl-N<sup>4</sup>-tetrahydrofuryl-2-methyl-p-phenylenediamine, N<sup>4</sup>-ethyl-N<sup>4</sup>-carboxymethyl-2-methyl-p-phenylenediamine, N<sup>4</sup>-carbamidomethyl-4'-ethyl-2-methyl-

VIII.

5



10 VIII-A.

15



20 IX.

30



IX-A.

35



**EXAMPLE 1**



X.

70

75

**EXAMPLE 2**

p-phenylenediamine, N<sup>4</sup>-ethyl-N<sup>4</sup>-tetrahydrofuryl-2-methyl-p-aminophenol, 3-acetylaminomethyl-4-aminodimethylaniline, N-ethyl-N- $\beta$ -methanesulfonamidoethyl-4-aminoaniline, N-ethyl-N- $\beta$ -methanesulfonamidoethyl-3-methyl-4-aminoaniline, the sodium salt of N-methyl-N- $\beta$ -sulfoethyl-p-phenylenediamine, etc.

The following examples demonstrate the stability of emulsions containing color formers prepared in accordance with our invention. The dyes hereinafter formulated will be referred to in the subsequent examples by the Roman numerals assigned to the dyes. In certain of the examples comparisons with other sensitizing dyes show the greatly superior stability of our new emulsions.

From the data in the above table it is apparent that two otherwise excellent red sensitizers (dyes VIII and IX) do not give emulsions which are sufficiently stable to be coated in the presence of color formers, whereas dyes VIII-A and IX-A give emulsions of satisfactory stability.

TABLE B

[Exposure through red filter which transmits substantially no light of wavelength shorter than 580 m $\mu$ .]

| Dye                                                                                                                                                                    | X     |          | X-A   |          | XI    |          | XI-A  |          |
|------------------------------------------------------------------------------------------------------------------------------------------------------------------------|-------|----------|-------|----------|-------|----------|-------|----------|
|                                                                                                                                                                        | Speed | $\gamma$ | Speed | $\gamma$ | Speed | $\gamma$ | Speed | $\gamma$ |
| gelatino-silver-bromiodide emulsion sensitized with dye <sup>1</sup>                                                                                                   | 63    | 1.76     | 63    | 2.11     | 480   | 1.87     | 240   | 1.98     |
| same gelatino-silver-bromio-iodide emulsion sensitized with same dye and containing a dispersion of an o-acylamino phenol coupler for cyan image                       | 13    | 0.26     | 4635  | 1.04     | 415   | 1.44     | 500   | 0.99     |
| same gelatino-silver-bromio-iodide emulsion sensitized with same dye and containing a dispersion of an o-acylamino phenol coupler for cyan image, held 1 hr. at 40°C.  | (2)   | —        | 55    | 1.07     | (2)   | —        | 480   | 1.09     |
| same gelatino-silver-bromio-iodide emulsion sensitized with same dye and containing a dispersion of an o-acylamino phenol coupler for cyan image, held 2 hrs. at 40°C. | (2)   | —        | 44.5  | 1.06     | (2)   | —        | 365   | 1.09     |

<sup>1</sup> Concentration of sensitizing dye was 30 mg. per liter of emulsion.<sup>2</sup> Red speed too low to measure.

From the data in the above Table B it is apparent that two otherwise excellent red sensitizers (dyes X and XI) do not give emulsions which are sufficiently stable to be coated in the presence of color formers, whereas dyes X-A and XI-A give emulsions of satisfactory stability.

30

## EXAMPLE 3

XII.



XIII.



TABLE C

[Exposure through a minus blue filter which transmits substantially no light of wavelength shorter than 500 m $\mu$ .]

| Dye                                                                                                                                                                | XII   |          | XIII  |          |
|--------------------------------------------------------------------------------------------------------------------------------------------------------------------|-------|----------|-------|----------|
|                                                                                                                                                                    | Speed | $\gamma$ | Speed | $\gamma$ |
| gelatino-silver-bromiodide emulsions sensitized with dye <sup>1</sup>                                                                                              | 160   | 0.58     | 370   | 1.58     |
| same gelatino-silver-bromio-iodide emulsion sensitized with same dye and containing a dispersion of a 5-pyrazolone coupler for magenta image, held 1 hr. at 40°C.  | 178   | 0.65     | 370   | 1.63     |
| same gelatino-silver-bromio-iodide emulsion sensitized with same dye and containing a dispersion of a 5-pyrazolone coupler for magenta image, held 2 hrs. at 40°C. | 3865  | 1.08     | —     | —        |

<sup>1</sup> Concentration of dye in all cases, 30 mg. per liter of emulsion.

## 11

The data in the above Table C show two yellow-green sensitizers either of which gives an emulsion containing a coupler for the magenta image, which emulsions are satisfactory for coating purposes.

## EXAMPLE 4

XIV.



TABLE D

[Exposure through red filter which transmits substantially no light of wavelength shorter than 580 m $\mu$ .]

| Dye                                                                                                                                                               | Speed | $\gamma$ |
|-------------------------------------------------------------------------------------------------------------------------------------------------------------------|-------|----------|
| gelatino-silver-bromiodide emulsion sensitized with dye XIV <sup>1</sup>                                                                                          | 185   | 0.44     |
| gelatino-silver-bromiodide emulsion sensitized with dye XIV and containing a dispersion of an o-acylaminophenol coupler for cyan image, held at 1 hr. for 40° C.  | 215   | 0.44     |
| gelatino-silver-bromiodide emulsion sensitized with dye XIV and containing a dispersion of an o-acylaminophenol coupler for cyan image, held at 2 hrs. for 40° C. | 185   | 0.43     |

<sup>1</sup> Concentration of sensitizing dye is 30 mg. per liter of emulsion in all cases.

In the above Table D it is shown that dye XIV gives a stable emulsion in the presence of color couplers for the cyan image.

## EXAMPLE 5

XV.



TABLE E

[Exposure through red filter which transmits substantially no light of wavelength shorter than 580 m $\mu$ .]

| Dye                                                                                                                                                                           | Speed | $\gamma$ |
|-------------------------------------------------------------------------------------------------------------------------------------------------------------------------------|-------|----------|
| gelatino-silver-bromiodide emulsion sensitized with dye XV <sup>1</sup>                                                                                                       | 645   | 0.48     |
| same gelatino-silver-bromiodide emulsion sensitized with same dye and containing a dispersion of an o-acylaminophenol color coupler for cyan image, held at 40° C. for 1 hr.  | 490   | 0.54     |
| same gelatino-silver-bromiodide emulsion sensitized with same dye and containing a dispersion of an o-acylaminophenol color coupler for cyan image, held at 40° C. for 2 hrs. | 370   | 0.55     |

<sup>1</sup> Concentration of dye in all cases, 30 mg. per liter of emulsion.

In the above Table E it is shown that dye XV gives a fairly stable emulsion in the presence of color couplers for the cyan image.

In preparing emulsions in accordance with our invention, the sensitizing dyes can be added to the emulsions in accordance with customary procedures, i. e. by adding a solution of the dye in an appropriate solvent to the emulsions. In the case of the dyes of Formulas II, III and IV, the dyes are advantageously dissolved in methyl alco-

## 12

hol and a volume of the methyl alcoholic solution (which may be diluted with water) containing from 5 to 100 mg. of the dye or dyes is slowly added to 1000 cc. of emulsion with stirring. In the case of the dyes of Formulas I, V, VI and VII, a water-soluble salt of the dyes is advantageously formed and dissolved in water, methyl alcohol or ethyl alcohol. The resulting solution of the water-soluble salt is then dispersed in the emulsions. The water-soluble salts are advantageously formed by adding to the dye or dyes (wet with a little water, methyl alcohol or ethyl alcohol), an alkali metal hydroxide, e. g. sodium or potassium hydroxide, or ammonium hydroxide, or an amine, e. g. methylamine, ethylamine, dimethylamine, diethylamine, trimethylamine, triethylamine, ethanolamine, diethanolamine, triethanolamine, pyridine, N-methylpiperidine, n-propylamine, isopropylamine, n-butylamine,  $\beta$ -ethoxyethylamine, etc. The salt which forms is then taken up in a suitable solvent, e. g. water, methyl alcohol, ethyl alcohol, a mixture of methyl alcohol and water, a mixture of ethyl alcohol and water, etc. As in the case of the dyes of Formulas II, III and IV, the dyes of Formulas I, V, VI and VII are ordinarily employed in a concentration of from 5 to 100 mg. per liter of emulsion. In the case of any of the sensitizing dyes employed in our invention, the optimum sensitizing effect is ordinarily obtained at a concentration of from 5 to 50 mg. of dye per liter of emulsion.

The sensitizing dyes in most cases should be added to the emulsions before the coupler of coupler dispersion is added.

The color-formers (couplers) are incorporated in the emulsions in the customary manner, e. g. by adding a dispersion of the coupler in a water-insoluble but water-permeable material (see above) to the emulsion, or by adding a dispersion of the alkali metal of the coupler in water. When employing dispersions of couplers in the aforesaid crystalloidal materials, the coupler (color former) which has been mixed with the high-boiling organic crystalloidal material to produce an oil-like mixture can be dispersed in water or gelatin solution or in any aqueous binder of colloidal character which is miscible with the silver halide emulsion. The dispersion can be effected with the aid of a homogenizer, colloid mill or the like, and the dispersions can be stabilized by the addition of emulsifying agents such as those of the well-known higher fatty alcohol sulfate type. The dispersion may also be formed by dispersing a solution of coupler and crystalloidal material in a solvent of low boiling point such as butyl acetate with water or gelatin solution and subsequently removing the low-boiling solvent by evaporation. Here also an emulsifying agent can be used. It is important that the mixture of coupler and crystalloidal material be a liquid at ordinary temperatures, so that liquid particles are formed when the mixture of coupler and crystalloidal material is emulsified in water and mixed with the emulsion, the particles retaining the coupler in solution, yet being readily penetrated by the photographic developing solution and other processing baths. The nature and proportions of the coupler and the crystalloidal material should be chosen so that the particles are liquid under the conditions of coating and processing the emulsion. With the aforesaid crystalloidal materials, there is little or no tendency to crystallization even when the coupler is present in a proportion amounting to 50% or more of the high-boiling crystalloidal material. The crystalloidal ma-

terials should also be substantially colorless and stable toward light, heat and moisture, in addition to being inert to the various processing baths which may be encountered, such as developers, oxidized developers, silver removal baths and fixing baths. They should have a sufficiently low refractive index so that solutions of the couplers in them have approximately the same refractive index as gelatin, thereby minimizing the opacity or light scattering of the coating. Most couplers themselves have high refractive indices and for this reason it is desirable that the oil formers have low refractive indices. The crystalloidal materials should be easily dispersible in the emulsions and should be chemically inert toward the couplers and dyes formed therefrom.

Our invention is directed primarily to the ordinarily employed gelatino-silver-halide developing-out emulsions, e. g., gelatino-silver-chloride, -chlorobromide, -chlorobromiodide, -iodochloride, -bromide and -bromiodide developing-out emulsions. These ordinarily employed silver halide developing out emulsions are emulsions which form "surface" latent image (see British Patent 581,772, accepted October 24, 1946). However, silver halide emulsions which form latent image mostly inside the silver halide grains (see British Patent 581,772 supra) can also be employed in practicing our invention.

The dyes set forth under Formula II above are described in the copending application of Leslie G. S. Brooker and Frank L. White, Serial No. 519,354, filed January 22, 1944, now U. S. Patent 2,478,366, issued August 9, 1949. The dyes set forth under Formula III above are described in United States Patent 2,213,238, dated September 3, 1940. The dyes set forth under Formula I above can be prepared as described in United States Patent 2,231,658, dated February 11, 1941, by condensing a cyclammonium carboxyalkyl quaternary salt containing a reactive methyl group with ethyl orthoformate, ethyl orthoacetate, ethyl orthopropionate, ethyl orthobutyrate or ethyl orthovalerate. The dyes set forth under Formulas IV-VIII above are prepared as described in the copending application of Gertrude Van Zandt and Leslie G. S. Brooker, Serial No. 711,816, filed November 22, 1946, now U. S. Patent 2,515,913, issued July 18, 1950.

What we claim as our invention and desire to be secured by Letters Patent of the United States is:

1. A red sensitive gelatino-silver-halide emulsion for color photography containing dispersed therein finely divided liquid particles of a mixture of a phenolic color-former for the cyan image capable of forming a quinoneimine dye with a phenylenediamine developer, and a substantially water-insoluble, low molecular weight, organic, crystalloidal material having a boiling point above about 175° C., said crystalloidal material having a high solvent action for the color former and for the dye formed therefrom, and being permeable to photographic processing solutions, the nature and proportions of the color former and crystalloidal material being so chosen that particles thereof are liquid under conditions of coating and processing the emulsion, said red sensitive emulsion being sensitized to the red with at least one sensitizing dye selected from the group consisting of those dyes represented by the following general formulas:



wherein D and D<sub>1</sub> each represents a divalent aliphatic hydrocarbon radical containing from 1 to 4 carbon atoms, R<sub>1</sub> and R<sub>4</sub> represent a member selected from the group consisting of a hydrogen atom and an alkyl group containing from 1 to 4 carbon atoms, Z and Z<sub>1</sub> each represents the non-metallic atoms necessary to complete a heterocyclic nucleus selected from the group consisting of heterocyclic nuclei of the benzothiazole series, heterocyclic nuclei of the benzoselenazole series, heterocyclic nuclei of the naphthothiazole series and heterocyclic nuclei of the naphthoselenazole series, R<sub>1</sub> and R<sub>3</sub> each represents an alkyl group containing from 1 to 2 carbon atoms, R<sub>2</sub> represents a monocyclic aryl group of the benzene series, and X represents an anion.

2. A yellow-green sensitive gelatino-silver-halide emulsion for color photography containing dispersed therein finely divided liquid particles of a mixture of a ketomethylene color-former for the magenta image capable of forming a quinoneimine dye with a phenylenediamine developer, and a substantially water-insoluble, low molecular weight, organic, crystalloidal material having a boiling point above about 175° C., said crystalloidal material having a high solvent action for the color former and for the dye formed therefrom, and being permeable to photographic processing solutions, the nature and proportions of the color former and crystalloidal material being so chosen that particles thereof are liquid under conditions of coating and processing the emulsion, said yellow-green sensitive emulsion being sensitized to the yellow-green with at least one sensitizing dye selected from the group consisting of those dyes represented by the following general formula:



15



wherein R<sub>4</sub> and R<sub>5</sub> each represents an alkyl group containing from 1 to 4 carbon atoms, X<sub>1</sub> represents an anion, D<sub>2</sub> and D<sub>3</sub> each represents a divalent aliphatic hydrocarbon radical containing from 1 to 4 carbon atoms, and Z<sub>3</sub> represents the non-metallic atoms necessary to complete a heterocyclic nucleus of the quinoline series.

3. A red sensitive gelatino-silver-halide emulsion for color photography containing dispersed therein finely divided liquid particles of a mixture of an o-acylaminophenol color-former for the cyan image capable of forming a quinoneimine dye with a phenylenediamine developer, and a substantially water-insoluble, low molecular weight, organic crystalloidal material having a boiling point above about 175° C., said crystalloidal material having a high solvent action for the color-former and for the dye formed therefrom, and being permeable to photographic processing solutions, the nature and proportions of the color-former and crystalloidal material being so chosen that particles thereof are liquid under conditions of coating and processing the emulsion, said red sensitive emulsion being sensitized to the red with at least one sensitizing dye selected from the group consisting of those dyes represented by the following general formulas:



wherein D and D<sub>1</sub> each represents a divalent aliphatic hydrocarbon radical containing from 1 to 4 carbon atoms, R and R<sub>4</sub> represent a member selected from the group consisting of a hydrogen atom and an alkyl group containing from 1 to 4 carbon atoms, Z and Z<sub>1</sub> each represents the non-metallic atoms necessary to complete a heterocyclic nucleus selected from the group consisting of heterocyclic nuclei of the benzothiazole series, heterocyclic nuclei of the benzoselenazole series, heterocyclic nuclei of the naphthothiazole series and heterocyclic nuclei of the naphthoselenazole series, R<sub>1</sub> and R<sub>3</sub> each represents an alkyl group containing from 1 to 2 carbon atoms, R<sub>2</sub> represents a monocyclic aryl group of the benzene series, and X represents an anion.

4. A red sensitive gelatino-silver-halide emulsion for color photography containing dispersed therein finely divided liquid particles of a mixture of an o-acylaminophenol color-former for the cyan image capable of forming a quinoneimine dye with a phenylenediamine developer, and a substantially water-insoluble, low molecular weight, organic crystalloidal material having a boiling point above about 175° C., said crystalloidal material having a high solvent action for the color-former and for the dye formed therefrom, and being permeable to photographic proc-

16

essing solutions, the nature and proportions of the color-former and crystalloidal material being so chosen that particles thereof are liquid under conditions of coating and processing the emulsion, said red sensitive emulsion being sensitized to the red with at least one sensitizing dye selected from the group consisting of those dyes represented by the following general formula:



wherein D represents a saturated divalent aliphatic hydrocarbon radical containing from 1 to 4 carbon atoms, R represents a member selected from the group consisting of a hydrogen atom and a primary alkyl group containing from 1 to 4 carbon atoms, and Z represents the non-metallic atoms necessary to complete a heterocyclic nucleus of the benzothiazole series.

5. A red sensitive gelatino-silver-halide emulsion for color photography containing dispersed therein finely divided liquid particles of a mixture of an o-acylaminophenol color-former for the cyan image capable of forming a quinoneimine dye with a phenylenediamine developer, and a substantially water-insoluble, low molecular weight, organic crystalloidal material having a boiling point above about 175° C., said crystalloidal material having a high solvent action for the color-former and for the dye formed therefrom and being permeable to photographic processing solutions, the nature and proportions of the color-former and crystalloidal material being so chosen that particles thereof are liquid under conditions of coating and processing the emulsion, said red sensitive emulsion being sensitized to the red with at least one sensitizing dye selected from the group consisting of those dyes represented by the following formula:



6. A red sensitive gelatino-silver-halide emulsion for color photography containing dispersed therein finely divided liquid particles of a mixture of an o-acylaminophenol color-former for the cyan image capable of forming a quinoneimine dye with a phenylenediamine developer, and a substantially water-insoluble, low molecular weight, organic crystalloidal material having a boiling point above about 175° C., said crystalloidal material having a high solvent action for the color-former and for the dye formed therefrom and being permeable to photographic processing solutions, the nature and proportions of the color-former and crystalloidal material being so chosen that particles thereof are liquid under conditions of coating and processing the emulsion, said red sensitive emulsion being sensitized to the red with at least one sensitizing dye selected from the group consisting of those dyes represented by the following general formula:



wherein R<sub>1</sub> represents an alkyl group containing from 1 to 2 carbon atoms, R<sub>2</sub> represents a mono-

17

cyclic aryl group of the benzene series; Z represents the non-metallic atoms necessary to complete a heterocyclic nucleus of the benzothiazole series; and X represents an anion.

7. A red sensitive gelatino-silver-halide emulsion for color photography containing dispersed therein finely divided liquid particles of a mixture of an o-acylaminophenol color-former for the cyan image capable of forming a quinone-imine dye with a phenylenediamine developer, and a substantially water-insoluble, low molecular weight, organic, crystalloidal material having a boiling point above about 175° C., said crystalloidal material having a high solvent action for the color-former and for the dye formed therefrom and being permeable to photographic processing solutions, the nature and proportions of the color-former and crystalloidal material being so chosen that particles thereof are liquid under conditions of coating and processing the emulsion, said red sensitive emulsion being sensitized to the red with at least one sensitizing dye selected from the group consisting of those dyes represented by the following formula:



8. A yellow-green sensitive gelatino-silver-halide emulsion for color photography containing dispersed therein finely divided liquid particles of a mixture of a 5-pyrazolone color-former for the magenta image capable of forming an azomethine dye with a phenylenediamine developer, and a substantially water-insoluble, low molecular weight, organic, crystalloidal material having a boiling point above about 175° C., said crystalloidal material having a high solvent action for the color-former and for the dye formed therefrom, and being permeable to photographic processing solutions, the nature and proportions of the color-former and crystalloidal material being so chosen that particles thereof are liquid under conditions of coating and processing the emulsion, said yellow-green sensitive emulsion being sensitized to the yellow-green with at least one sensitizing dye selected from the group consisting of those dyes represented by the following general formulas:



18



wherein R4 and R5 each represents an alkyl group containing from 1 to 4 carbon atoms; X1 represents an anion; D2 and D3 each represents a divalent aliphatic hydrocarbon radical containing from 1 to 4 carbon atoms; and Z3 represents the non-metallic atoms necessary to complete a heterocyclic nucleus of the quinoline series.

20. 9. A yellow-green sensitive gelatino-silver-halide emulsion for color photography containing dispersed therein finely divided liquid particles of a mixture of a 5-pyrazolone color-former for the magenta image capable of forming an azomethine dye with a phenylenediamine developer, and a substantially water-insoluble, low molecular weight, organic, crystalloidal material having a boiling point above about 175° C., said crystalloidal material having a high solvent action for the color-former and for the dye formed therefrom, and being permeable to photographic processing solutions, the nature and proportions of the color-former and crystalloidal material being so chosen that particles thereof are liquid under conditions of coating and processing the emulsion, said yellow-green sensitive emulsion being sensitized to the yellow-green with at least one sensitizing dye selected from the group consisting of those dyes represented by the following general formula:



55. 10. A yellow-green sensitive gelatino-silver-halide emulsion for color photography containing dispersed therein finely divided liquid particles of a mixture of a 5-pyrazolone color-former for the magenta image capable of forming an azomethine dye with a phenylenediamine developer, and a substantially water-insoluble, low molecular weight, organic, crystalloidal material having a boiling point above about 175° C., said crystalloidal material having a high solvent action for the color-former and for the dye formed therefrom, and being permeable to photographic processing solutions, the nature and proportions of the color-former and crystalloidal material being so chosen that particles thereof are liquid under conditions of coating and processing the emulsion, said yellow-green sensitive emulsion being sensitized to the yellow-green with at least one sensitizing dye selected from the group consisting of those dyes represented by the following general formulas:

56. 11. A yellow-green sensitive gelatino-silver-halide emulsion for color photography containing dispersed therein finely divided liquid particles of a mixture of a 5-pyrazolone color-former for the magenta image capable of forming an azomethine dye with a phenylenediamine developer, and a substantially water-insoluble, low molecular weight, organic, crystalloidal material having a boiling point above about 175° C., said crystalloidal material having a high solvent action for the color-former and for the dye formed therefrom, and being permeable to photographic processing solutions, the nature and proportions of the color-former and crystalloidal material being so chosen that particles thereof are liquid under conditions of coating and processing the emulsion, said yellow-green sensitive emulsion being sensitized to the yellow-green with at least one sensitizing dye selected from the group consisting of those dyes represented by the following general formulas:

75. 12. A yellow-green sensitive gelatino-silver-halide emulsion for color photography containing dispersed therein finely divided liquid particles of a mixture of a 5-pyrazolone color-former for the magenta image capable of forming an azomethine dye with a phenylenediamine developer, and a substantially water-insoluble, low molecular weight, organic, crystalloidal material having a boiling point above about 175° C., said crystalloidal material having a high solvent action for the color-former and for the dye formed therefrom, and being permeable to photographic processing solutions, the nature and proportions of the color-former and crystalloidal material being so chosen that particles thereof are liquid under conditions of coating and processing the emulsion, said yellow-green sensitive emulsion being sensitized to the yellow-green with at least one sensitizing dye selected from the group consisting of those dyes represented by the following general formulas:

ing so chosen that particles thereof are liquid under conditions of coating and processing the emulsion, said yellow-green sensitive emulsion being sensitized to the yellow-green with at least one sensitizing dye selected from the group consisting of those dyes represented by the following formula:



11. A sensitive silver halide emulsion for color photography selected from the group consisting of (I) a red sensitive silver halide emulsion containing dispersed therein finely divided liquid particles of a mixture of a phenolic color-former for the cyan image capable of forming a quinone-imine dye with a phenylenediamine developer, and a substantially water-insoluble, low molecular weight, organic, crystallloid material having a boiling point above about 175° C., said crystallloid material having a high solvent action for the color-former and for the dye formed therefrom, and being permeable to photographic processing solutions, the nature and proportions of the color-former and crystallloid material being so chosen that particles thereof are liquid under conditions of coating and processing the emulsion, said red sensitive emulsion being sensitized to the red with at least one sensitizing dye selected from the group consisting of those dyes represented by the following general formulas:



wherein D and D<sub>1</sub> each represents a divalent aliphatic hydrocarbon radical containing from 1 to 4 carbon atoms, R and R<sub>4</sub> represent a member selected from the group consisting of a hydrogen atom and an alkyl group consisting from 1 to 4 carbon atoms, Z and Z<sub>1</sub> each represents the non-metallic atoms necessary to complete a heterocyclic nucleus selected from the group consisting of heterocyclic nuclei of the benzothiazole series, heterocyclic nuclei of the benzoselenazole series, heterocyclic nuclei of the naphthothiazole series and heterocyclic nuclei of the naphthoselenazole series, R<sub>1</sub> and R<sub>3</sub> each represents an alkyl group containing from 1 to 2 carbon atoms, R<sub>2</sub> represents a monocyclic aryl group of the benzene series, and X represents an anion, and (II) a yellow-green sensitive silver halide emulsion containing dispersed therein finely divided liquid particles of a mixture of a ketomethylene color-former for the magenta image capable of forming a quinoneimine dye with a phenylenediamine developer, and a substantially water-insoluble,

low molecular weight, organic, crystalloidal material having a boiling point above about 175°C., said crystalloidal material having a high solvent action for the color-former and for the dye formed therefrom, and being permeable to photographic processing solutions, the nature and proportions of the color-former and crystalloidal material being so chosen that particles thereof are liquid under conditions of coating and processing the emulsion, said yellow-green sensitive silver halide emulsion being sensitized to the yellow-green with at least one sensitizing dye selected from the group consisting of those dyes represented by the following general formulas:



50 wherein  $R_4$  and  $R_5$  each represents an alkyl group containing from 1 to 4 carbon atoms,  $X_1$  represents an anion,  $D_2$  and  $D_3$  each represents a divalent aliphatic hydrocarbon radical containing from 1 to 4 carbon atoms, and  $Z_3$  represents the non-metallic atoms necessary to complete a heterocyclic nucleus of the quinoline series.

JOHN SPENCE.  
BURT H. CARROLL.

References Cited in the file of this patent

UNITED STATES PATENTS

| Number    | Name             | Date          |
|-----------|------------------|---------------|
| 2,148,979 | Dieterle         | Feb. 28, 1939 |
| 2,148,980 | Dieterle         | Feb. 28, 1939 |
| 2,213,238 | Brooker et al.   | Sept. 3, 1940 |
| 2,231,658 | Brooker et al.   | Feb. 11, 1941 |
| 2,304,940 | Mannes et al.    | Dec. 15, 1942 |
| 2,322,027 | Jelley et al.    | June 15, 1943 |
| 2,478,366 | Brooker et al.   | Aug. 9, 1949  |
| 2,515,913 | Van Zandt et al. | July 18, 1950 |